

## UNITED STATES PATENT OFFICE

WINFRID HENTRICH AND MAX HARDTMANN, OF WIESDORF, PETER BACKES, OF COLOGNE-DEUTZ, AND HERMANN STÖTTER, OF LEVERKUSEN-ON-THE-RHINE, GERMANY, ASSIGNOR TO I. G. FARBENINDUSTRIE AKTIENGESELLSCHAFT, OF FRANKFORT-ON-THE-MAIN, GERMANY, A CORPORATION OF GERMANY

## TEXTILE PEST PROOFING MEDIA

No Drawing. Application filed July 18, 1930, Serial No. 468,442, and in Germany August 26, 1929.

The present invention relates to new media for protecting wool, furs, feathers, hair and the like from attack by moths or damage by other textile pests.

5 In accordance with the invention materials liable to attack by moths or other animal textile pests, such as hair, feathers, furs, wool and the like can be protected from the attack by such pests by incorporating therewith an inorganic selenium compound such as selenious acid, selenic acid and salts thereof.

10 The compounds coming into consideration for the purpose of our invention are generally in the form of their salts colorless crystalline compounds soluble in water and may be prepared, for example, according to the statements of Berichte der deutschen chemischen Gesellschaft, vol. 55, page 2082; 15 Zeitschrift für anorganische Chemie, vol. 116, page 193 and vol. 140, page 47. By way of example the following compounds may be mentioned: selenious acid, selenic acid, sodium selenate, ammonium selenite, selenious acid ethylene diamine and the like.

20 The protecting agents can be applied in various ways and even small proportions, for instance, 0.1-2 per cent applied to the materials to be protected may have the desired effect. Thus, for example, the compounds soluble in organic solvents can be dissolved in appropriate solvents, such as alcohols, acetone, cyclohexanone and the like and sprayed on to the materials to be protected, 25 or the materials may be steeped into the solutions of the active substances, or the materials may be otherwise wetted. Conversely, the water soluble compounds (in the free form or as water soluble salts) can be caused 30 to act on the materials to be treated in an aqueous solution, in which connection the addition of organic or inorganic salts or acids or also of wetting agents may be advantageous. Obviously the materials can also 35 be simultaneously dyed and impregnated and when dyed with sulfuric acid it is possible to replace the sulfuric acid by selenic acid  $H_2SeO_4$ . According to the nature of the 40 materials to be treated other methods of impregnation can also be employed and will 45

readily suggest themselves. The protective agent is tenaciously retained by the objects thus treated, which thereby are protected from attack by textile pests.

55 The following examples serve to illustrate our invention without limiting it thereto:

Example 1.—100 kgs. of wool are treated for half an hour in the manner of a dyeing process with 1 kg. of selenic acid in the usual way with or without addition of a dyestuff. Then the material is rinsed, hydroextracted and dried. The wool is now protected 60 against attack by moths, *anthrenus*, *attagenus* and other textile pests.

65 Example 2.—The materials to be protected are treated for some time with a cold solution containing 1-2 grams per liter of selenious acid, then rinsed with water and dried. The materials show the same effect 70 as described in Example 1.

75 Example 3.—The wool to be protected is treated for some time with a cold aqueous solution containing 1-1.5 grams per liter of ammonium selenate. The material is then centrifuged and dried. The wool is thus rendered moth proof.

80 Example 4.—The material to be protected is treated for some time with a cold aqueous solution containing 1-1.5 grams per liter of ammonium selenite. After hydroextracting the materials are dried. The protection against textile pests is the same as described before.

85 Example 5.—Wool is impregnated with an aqueous solution containing 1-1.5 grams per liter of selenious acid ethylene diamine. After some time it is centrifuged and dried. The wool is thus rendered moth proof.

90 Example 6.—Wool is treated with a solution of 1.5 parts by weight of selenious acid in 100 parts by weight of an organic solvent. By this treatment the wool is permanently protected from attack by moths and the like.

95 Instead of the selenious acid other selenium compounds, soluble in organic solvents, can also be used in a similar manner, for example, salts of selenious acid with organic bases, for instance, with ethylenediamine, *n*-butylamine, cyclohexylamine and the like. All 100

these compounds, even in small proportions, confer upon the materials treated therewith an excellent protection against attack by textile pests.

5 *Example 7.*—100 kilograms of wool are treated in the manner of a dyeing process with 0.5 per cent of ammonium selenate and 4 per cent of sulfuric acid. By this treatment the wool shows the formerly described effect.

10 *Example 8.*—100 grams of wool are treated in the manner of a dyeing process while boiling with 6 per cent of naphthyl amine black (Colour Index, 1924 number 246), 10 per cent of Glauber's salt ( $\text{Na}_2\text{SO}_4$ ) and 4 per cent of selenic acid. The material thus treated is permanently protected against attack by moths, *anthrenus*, *attagenus* and other textile pests.

15 20 We claim:

1. A textile pest proofing medium containing a water soluble salt of selenic acid.

2. A moth proofing medium containing the sodium selenate of the formula:  $\text{SeO}_4\text{Na}_2$ .

25 3. A textile pest-proofing agent containing a water-soluble compound of the formula



30 wherein  $n$  is 3 or 4, and X stands for hydrogen, alkali metal, or ammonium which may be substituted by an organic radical.

35 In testimony whereof, we affix our signatures.

WINFRID HENTRICH.  
MAX HARDTMANN.  
PETER BACKES.  
HERMANN STÖTTER.

40

45

50

55

60

65